# EUROPEAN PATENT APPLICATION

(11) **EP 1 674 552 A1**
(43) Date of publication of application: **28.06.2006**
(21) Application number: 04258148.8
(22) Date of filing: 24.12.2004
(51) Int. Cl.: C10L 1/02, C10L 1/18

(54) **Fuel compositions**

(71) Applicant: SHELL INTERNATIONALE RESEARCH MAATSCHAPPIJ B.V., 2596 HR Den Haag (NL)
(72) Inventor: The designation of the inventor has not yet been filed

(57) **Abstract**

The invention provides a diesel fuel composition containing a diesel base fuel and a palm oil alkyl ester (POAE), wherein the POAE concentration is up to 25 % v/v based on the overall composition. Further provided is the use of a POAE in a diesel fuel composition for the purpose of improving its cold flow performance. The POAE is preferably used at a concentration, between 0 and 100 % v/v based on the overall fuel composition, at which its ability to reduce the cold filter plugging point of the composition reaches a maximum.

## Description

This invention relates to diesel fuel compositions, their preparation and their uses, as well as to the use of a particular fuel component for a new purpose.

It is known to include fatty acid alkyl esters (FAAEs), in particular fatty acid methyl esters, in diesel fuel compositions. They are typically derivable from biological sources and can be used to reduce the environmental impact from production and use of a conventional petrol-derived fuel.

The most common such additive is rapeseed methyl ester (RME), which has already been used in commercially available diesel fuels.

There is increasing pressure, both from regulatory bodies and also from consumers, to increase the use of such "biofuels" so as to improve the environmental effects of using automotive fuels. However the inclusion of a FAAE can in certain contexts be detrimental to the properties of the overall composition. In particular, fatty acid methyl esters (FAMEs) are well known to have poor cold flow properties compared to typical diesel base fuels (as evidenced by their relatively high cold filter plugging points, CFPPs), and it would therefore be expected that when added to another diesel fuel they would impair its low temperature performance. This effect has indeed been observed in many base fuel/FAME blends.

Following conventional fuel formulation principles, it would also be expected that the cold flow performance of a diesel base fuel/FAAE blend, as evidenced for instance by its CFPP, would vary linearly with FAAE concentration. In other words, the addition of a FAAE to a fuel having a lower CFPP would be expected to increase the CFPP of the fuel to an extent directly proportional to the amount of FAAE added.

It has now been surprisingly discovered that one of the FAAEs, palm oil methyl ester (POME), can actually improve the cold flow performance of a diesel fuel composition in particular when present at concentrations of up to 25 % v/v.

According to a first aspect of the present invention there is therefore provided a diesel fuel composition containing a palm oil alkyl ester (POAE), wherein the POAE concentration is up to 25 % v/v based on the overall composition.

Preferably the POAE concentration is greater than 5 % v/v; more preferably it is 8 or 10 % v/v or greater.

Typically the composition will contain, in addition to the POAE, a major proportion of a diesel base fuel. In this context a "major proportion" means suitably 70 % v/v or greater, preferably 75 or 80 % v/v or greater, in cases up to 85 or 90 % v/v or greater.

By "palm oil alkyl ester" or "POAE" is meant an alkyl ester of an oil derived from either the fruit or the seed (preferably the fruit) of *Elaeis guineensis* Jacq., *Palmae*. This palm oil will chiefly comprise palmitin, with some quantities of stearin and linolein. The alkyl ester may be synthesised for instance by esterification (typically base-catalysed, such as by KOH) of the palm oil with a suitable alcohol; for example, the methyl ester can be synthesised by esterification with methanol.

Preferably the POAE will be a C₁ to C₅ alkyl ester, more preferably either the methyl, ethyl or propyl (suitably iso-propyl) ester, yet more preferably either the methyl or ethyl ester. Most preferably it will be palm oil methyl ester (POME).

The POAE suitably complies with specifications applying to the base fuel which forms the major proportion of the fuel composition, bearing in mind the intended use to which the composition is to be put (for example, in which geographical area and at what time of year). In particular, the POAE preferably has a flash point (IP 34) of greater than 101 °C; a kinematic viscosity at 40 °C (IP 71) of 1.9 to 6.0 centistokes, preferably 3.5 to 5.0 centistokes; a density from 845 to 910 kg/m³, preferably from 860 to 900 kg/m³, at 15 °C (IP 365, EN ISO 12185 or EN ISO 3675); a water content (IP 386) of less than 500 ppmw (parts per million by weight); a T95 (the temperature at which 95 % of the fuel has evaporated, measured according to IP 123) of less than 360 °C; an acid number (IP 139) of less than 0.8 mgKOH/g, preferably less than 0.5 mgKOH/g; and an iodine number (IP 84) of less than 125, preferably less than 120 or less than 115, grams of iodine (I₂) per 100 g of fuel. It also preferably contains (eg, by NMR) less than 0.2 % w/w of free methanol, less than 0.02 % w/w of free glycerol and greater than 96.5 % w/w esters. In general it may be preferred for the POAE to conform to the European specification EN 14214 for fatty acid methyl esters for use as diesel fuels.

The cold filter plugging point of the POAE (IP 309) is suitably from +10 to +15 °C, such as from +11 to +14 °C.

The POAE may be included in the composition with one or more other fatty acid alkyl esters, in particular fatty acid methyl esters, which may be pre-blended with the POAE or added to the fuel composition separately.

The concentration of the POAE in the fuel composition is preferably up to 22 % v/v, based on the overall fuel composition, more preferably up to 20 % v/v and most preferably up to 15 % v/v. Its concentration may be as low as 15 % v/v, in cases as low as 13 %, 12.5 %, 12 %, 11 %, 10 % or 7.5 % v/v, or in cases as low as 6 %, 5 %, 3 %, 2 % or even 1 % v/v.

In particular the POAE concentration may suitably be from 5 to 20 % v/v, more preferably from 7.5 to 15 or 20 % v/v such as from 10 to 15 % v/v based on the overall composition.

The diesel base fuel used in a composition according to the invention may be any known diesel base fuel, and it may itself comprise a mixture of diesel fuel components. It will preferably have a sulphur content of at most 2000 ppmw (parts per million by weight). More preferably it will have a low or ultra low sulphur content, for instance at most 500 ppmw, preferably no more than 350 ppmw, most preferably no more than 100 or 50 or 30 or even 10 ppmw, of sulphur. The fuel composition after addition of the POAE will also preferably have a sulphur content within these ranges.

In some cases it may however be preferred that the base fuel is not a sulphur-free ("zero sulphur") fuel.

Typical diesel fuel components comprise liquid hydrocarbon middle distillate fuel oils, for instance petroleum derived gas oils. Such base fuel components may be organically or synthetically derived. They will typically have boiling points within the usual diesel range of 150 to 400 °C, depending on grade and use. They will typically have densities from 0.75 to 0.9 g/cm³, preferably from 0.8 to 0.86 g/cm³, at 15 °C (IP 365) and cetane numbers (ASTM D613) of from 35 to 80, more preferably from 40 to 75. Their initial boiling points will suitably be in the range 150 to 230 °C and their final boiling points in the range 290 to 400 °C. Their kinematic viscosity at 40 °C (IP 71) might suitably be from 1.5 to 4.5 centistokes.

Again, the fuel composition of the invention, which includes the POAE, will also preferably fall within these general specifications.

Such fuels are generally suitable for use in a compression ignition (diesel) internal combustion engine, of either the indirect or the direct injection type.

It may be preferred for the base fuel to be an ultra low sulphur fuel (ie, no more than 50 ppmw sulphur), and/or for it to contain no refinery additives, or at least no additional cold flow additives. It will preferably be a "summer grade" fuel, and/or be suitable and/or intended for use in climates unlikely to suffer extremely low temperatures. This applies for example where the ambient temperature is unlikely to fall below - 6 or even -8 °C. Diesel fuels for use in New Zealand, for instance, currently need only comply with a cold filter plugging point (CFPP) specification down to -6 °C, for South Africa compliance is only necessary to -4 °C and for some regions of China a CFPP between +4 and +12 °C is considered acceptable. In diesel fuel compositions intended for this type of use, the present invention can make it possible to use the POAE as a substitute (either complete or partial) for conventional cold flow additives, as will be described below.

A petroleum derived gas oil may be obtained from refining and optionally (hydro)processing a crude petroleum source. It may be a single gas oil stream obtained from such a refinery process or a blend of several gas oil fractions obtained in the refinery process via different processing routes. Examples of such gas oil fractions are straight run gas oil, vacuum gas oil, gas oil as obtained in a thermal cracking process, light and heavy cycle oils as obtained in a fluid catalytic cracking unit and gas oil as obtained from a hydrocracker unit. Optionally a petroleum derived gas oil may comprise some petroleum derived kerosene fraction.

Such gas oils may be processed in a hydrodesulphurisation (HDS) unit so as to reduce their sulphur content to a level suitable for inclusion in a diesel fuel composition.

In a composition according to the invention, the base fuel may be or contain another so-called "biodiesel" fuel component, such as an alcohol (in particular methanol or ethanol) or other oxygenate or a vegetable oil or vegetable oil derivative other than a POAE.

It may be or contain a Fischer-Tropsch derived fuel, in particular a Fischer-Tropsch derived gas oil. Such fuels are known and in use in diesel fuel compositions. They are, or are prepared from, the synthesis products of a Fischer-Tropsch condensation reaction, as for example the commercially used gas oil obtained from the Shell Middle Distillate Synthesis (Gas To Liquid) process operating in Bintulu (Malaysia).

In general a diesel fuel composition according to the invention may contain no, or only low levels of, other cold flow additives such as flow improvers and wax anti-settling agents. A "low level" in this context is suitably 200 ppmw or less, preferably 100 or 50 ppmw or less, yet more preferably 25 or 10 or 5 ppmw or less.

Subject to the above, the composition of the invention may contain other components in addition to the diesel base fuel and the POAE. Typically such components will be incorporated in fuel additives. Examples include detergents such as polyolefin substituted succinimides or succinamides of polyamines, for instance polyisobutylene succinimides or polyisobutylene amine succinamides, aliphatic amines, Mannich bases or amines and polyolefin (eg, polyisobutylene) maleic anhydrides (suitable detergents can be obtained from Infineum (eg, F7661 and F7685) and Octel (eg, OMA 4130D)); lubricity enhancers such as EC 832 and PARADYNE™ (ex Infineum), HITEC™ E580 (ex Ethyl Corporation) and VEKTRON™ 6010 (ex Infineum) and amide-based additives such as those available from the Lubrizol Chemical Company, for instance LZ 539 C; dehazers, eg, alkoxylated phenol formaldehyde polymers such as those commercially available as NALCO™ EC5462A (formerly 7D07) (ex Nalco), and TOLAD™ 2683 (ex Petrolite); anti-foaming agents (eg, the polyether-modified polysiloxanes commercially available as TEGOPREN™ 5851 and Q 25907 (ex Dow Corning), SAG™ TP-325 (ex OSi) and RHODORSIL™ (ex Rhone Poulenc)); ignition improvers (cetane improvers) (eg, 2-ethylhexyl nitrate (EHN), cyclohexyl nitrate, di-tert-butyl peroxide and those disclosed in US-4,208,190 at column 2, line 27 to column 3, line 21); anti-rust agents (eg, that sold commercially by Rhein Chemie, Mannheim, Germany as "RC 4801", a propane-1, 2-diol semi-ester of tetrapropenyl succinic acid, or polyhydric alcohol esters of a succinic acid derivative, the succinic acid derivative having on at least one of its alpha-carbon atoms an unsubstituted or substituted aliphatic hydrocarbon group containing from 20 to 500 carbon atoms, eg, the pentaerythritol diester of polyisobutylene-substituted succinic acid); corrosion inhibitors; reodorants; anti-wear additives; anti-oxidants (eg, phenolics such as 2,6-di-tertbutylphenol, or phenylenediamines such as N,N'-di-sec-butyl-p-phenylenediamine); metal deactivators; and combustion improvers.

The fuel composition will suitably contain only a minor amount of such additives. Thus unless otherwise stated, the (active matter) concentration of each such additional component in the overall fuel composition is preferably up to 1 % w/w, more preferably in the range from 5 to 1000 ppmw, advantageously from 75 to 300 ppmw, such as from 95 to 150 ppmw.

It may be preferred that a lubricity enhancer be included in the composition, especially when it has a low (eg, 500 ppmw or less) sulphur content. The lubricity enhancer is conveniently present at a concentration from 50 to 1000 ppmw, preferably from 100 to 1000 ppmw, based on the overall fuel composition. However since the POAE may itself help to improve lubricity, lower levels of lubricity enhancer may be sufficient.

Additives may be added at various stages during the production of a fuel composition; those added at the refinery for example might be selected from anti-static agents, pipeline drag reducers and (subject to the above comments) flow improvers (eg, ethylene/vinyl acetate copolymers or acrylate/maleic anhydride copolymers) and wax anti-settling agents (eg, those commercially available under the trade marks "OCTEL" (eg, OCTEL™ W 5000, ex Octel) and "DODIFLOW" (eg, DODIFLOW™ v 3958, ex Hoechst) or as R474 (ex Infineum)). Other additives may be added downstream of the refinery.

According to a second aspect of the present invention, there is provided the use of a POAE in a diesel fuel composition, for the purpose of improving the cold flow performance of the composition.

In the context of this second aspect of the invention, "use" of a POAE in a diesel fuel composition means incorporating the POAE into the composition, typically as a blend (ie, a physical mixture) with one or more other fuel components and optionally with one or more fuel additives. The POAE is conveniently incorporated before the composition is introduced into an internal combustion engine or other system which is to be run on the composition. Instead or in addition the use may involve running a diesel engine on the fuel composition containing the POAE, typically by introducing the composition into a combustion chamber of the engine.

"Improving" embraces any degree of improvement compared to the cold flow performance of the fuel composition before the POAE is added.

As described above, it is surprising that a POAE can act to improve the cold flow performance of a diesel fuel composition. It is well known that certain fatty acid alkyl esters have poor cold flow properties compared with typical diesel base fuels. For example, the cold filter plugging point (CFPP) of palm oil methyl ester (POME) is +10 to +15 °C, typically ~ 11 °C, as compared to -6 to -8 °C for a typical ultra low sulphur diesel base fuel without cold flow additives. Unexpectedly, however, it has now been found that the addition of certain quantities of a POAE (in particular POME) to a diesel base fuel can actually suppress the CFPP of the fuel. In other words, the increase in CFPP with increasing POAE concentration is non-linear, beginning at lower POAE concentrations with a beneficial effect. This effect has not been observed with other fatty acid alkyl esters tested, for example RME.

Indeed it has been found that for a diesel base fuel/POME blend, normal "linear blending rules" do not apply to the change in cold flow performance with POME concentration. At lower concentrations the POME can actually reduce the CFPP of the base fuel despite the fact that its own CFPP is higher than that of the base fuel. If linear blending rules applied then the CFPP of the blend would increase linearly with increasing POME concentration.

As a result of this discovery, the present invention is able to provide a more optimised method for improving the cold flow performance (ie, reducing the CFPP) of a diesel fuel composition to reach a particular target value, as will be further described in connection with the third aspect of the invention.

The invention moreover makes possible - and indeed desirable - the use of a POAE in a diesel fuel composition, often at higher concentrations than have previously been thought suitable. This can bring other benefits in addition to the improvement in cold flow performance, for example improved lubricity performance (it is already known to add fatty acid alkyl esters to diesel fuel compositions for this purpose), a reduction in life cycle greenhouse gas emissions and potentially reduced costs in particular compared to the use of other available "biofuels" such as RME.

The cold flow performance of the fuel composition is suitably assessed by measuring its cold filter plugging point (CFPP), preferably using the standard test method IP 309 or an analogous technique. The CFPP of a fuel indicates the temperature at and below which wax in the fuel will cause severe restrictions to flow through a filter screen, and correlates well with vehicle operability at lower temperatures. An improvement in cold flow performance will correspond to a reduction in the CFPP.

Preferably, by using the invention, the CFPP of the composition is reduced by at least 1 °C compared to its value prior to addition of the POAE, more preferably by at least 2 °C, yet more preferably by at least 3 °C and most preferably by at least 4 °C. Preferably, by using the invention, the CFPP of the composition is reduced by at least 0.3 % of its value (expressed in Kelvin) prior to addition of the POAE, more preferably by at least 0.5 or 0.7 % and most preferably by at least 1 or 1.2 or 1.5 or even 1.6 %.

The POAE is preferably used in the fuel composition at a concentration of up to 25 % v/v, based on the overall fuel composition after POAE addition, more preferably at a concentration of up to 22 % v/v, yet more preferably at up to 20 % v/v and most preferably at up to 15 % v/v. It may be used at a concentration of as low as 12 %, 10 % or 7.5 % v/v, or in cases as low as 6 %, 5 %, 3 %, 2 % or even 1 % v/v.

In particular the POAE may suitably be used at a concentration of from 5 to 20 % v/v, more preferably from 7.5 to 15 or 20 % v/v, such as from 10 to 15 % v/v, based on the overall fuel composition after POAE addition.

The fuel composition, prior to addition of the POAE, suitably comprises a major proportion of a diesel base fuel. By "major proportion" here is meant typically 80 % v/v or greater, suitably 90 or 95 % v/v or greater; most preferably 98 or 99 or 99.5 % v/v or greater or in cases 100 %. At its simplest therefore, the composition which results from carrying out the present invention will contain only the diesel base fuel and the POAE; the invention thus embraces the addition of a POAE to a diesel base fuel so as to improve its cold flow properties, and the improvement may be with respect to the properties of the base fuel alone. However the composition may contain other components, in particular diesel fuel additives, as described above in connection with the first aspect of the invention.

In general the composition which results from the method of the invention may contain no, or only low levels of, other cold flow additives. A "low level" in this context is suitably 200 ppmw or less, preferably 100 or 50 ppmw or less, yet more preferably 25 or 10 or 5 ppmw or less.

The invention thus embraces the use of a POAE in a diesel fuel composition for the purpose of reducing the level of cold flow additives in the composition. Here the term "reducing" embraces reduction to zero; in other words, the POAE may be used to replace one or more cold flow additives either partially or completely. The reduction may be as compared to the level of the relevant additive(s) which would otherwise have been incorporated into the fuel composition in order to achieve a desired target CFPP, for instance in order to meet government fuel specifications or consumer expectations. Thus the POAE can help in reducing the overall additive levels in the composition and their associated costs.

Preferably the POAE is used to reduce the w/w concentration of the relevant additive(s) in the fuel composition by at least 10 %, more preferably by at least 20 or 30 %, yet more preferably by at least 50 or 70 or 80 or even 90 % or, as described above, by 100 %.

It may for instance be used to replace cold flow additive(s) to an extent that the concentration of cold flow additives remaining in the fuel composition is 300 ppmw or less, preferably 200 ppmw or less, more preferably 100 or 50 ppmw or less. Most preferably it may be used to replace cold flow additive(s) substantially entirely, the fuel composition being nearly or essentially free of such additives and containing for example 10 or 5 ppmw or less, preferably 1 ppmw or less, of cold flow additives.

(All additive concentrations quoted in this specification refer, unless otherwise stated, to active matter concentrations by mass. The term "cold flow additive" refers to an additive, other than the POAE, which improves the low temperature performance of a fuel (eg, lowering its CFPP).)

Again it may be preferred for the fuel composition to contain no, or only low levels of, refinery additives other than cold flow additives.

When carrying out the method of the second aspect of the invention, the POAE may be used in the fuel composition for one or more other purposes in addition to the desire to improve cold flow performance, for instance to reduce environmental impact, to improve lubricity and/or to reduce costs. In such cases it may be sufficient, for the purposes of the invention, that the cold flow performance of the resultant fuel composition be no worse than, or not substantially worse than, the cold flow performance of the composition before addition of the POAE; in other words the cold flow performance of the composition is maintained alongside the other purposes achieved by addition of the POAE.

In this context "maintenance" of the cold flow properties may mean that the CFPP of the composition is not increased by more than 1 % of its value (in Kelvin) prior to addition of the POAE, preferably not by more than 0.75 or 0.5 % and most preferably not by more than 0.2 or even 0.1 or 0.05 %. It may mean that the CFPP of the composition is not increased by more than 3 °C, preferably not by more than 2 °C, most preferably not by more than 1 or 0.5 °C, compared to its value prior to addition of the POAE.

The present invention therefore also embraces the use of a POAE in a diesel fuel composition for two or more simultaneous purposes, one of which is to maintain the CFPP of the composition below a certain desired level. This desired level may be the CFPP of the composition prior to addition of the POAE.

According to a third aspect, the present invention provides a method for altering (typically reducing) the CFPP of a diesel fuel composition which contains a major proportion of a diesel base fuel, in order to reach a target CFPP X, which method comprises adding to the base fuel an amount x of a POAE having a CFPP B which is higher than the CFPP A of the base fuel, wherein x is greater than the amount of POAE which could be added to the base fuel, without exceeding the target CFPP X, if linear blending rules applied.

As described above, if linear blending rules applied it would be straightforward to calculate the maximum amount of a POAE which could be added to the base fuel before exceeding a given target CFPP. However it has now been found that, in particular at concentrations below about 45 % v/v, a POAE can act to depress the CFPP of a diesel base fuel below the level that would be expected if linear blending rules applied. This allows a higher amount of a POAE to be included in a diesel fuel composition which has to meet any given target CFPP. Since there may be other advantages, as described above, to including higher POAE levels, the ability to do so without undue detriment to the cold flow performance of the composition can provide formulation advantages.

In the context of the third aspect of the invention a "major proportion" of a base fuel means typically 80 % v/v or greater, more suitably 90 or 95 % v/v or greater, yet more suitably 98 or 99 or 99.5 % v/v or greater or in cases 100 %. "Reaching" a target CFPP generally means attaining a CFPP at or below the target value.

The POAE will typically be added to the base fuel as a blend (ie, a physical mixture), conveniently before the overall composition is introduced into an internal combustion engine or other system which is to be run on the composition. Other fuel components and/or fuel additives may also be incorporated into the composition, either before or after addition of the POAE and either before or during use of the composition in a combustion system.

The amount of POAE added will depend on the natures of the base fuel and POAE and on the target CFPP. In general, the volume fraction v of the POAE in the resultant base fuel/POAE mixture will be greater than the volume fraction v' which would be suitable if linear blending rules applied, wherein v' would be defined by the equation : $X = A + {v}^{′} ( B - A ) .$
The volume fractions v and v' must each have a value between 0 and 1. When carrying out the method of the invention the actual volume fraction of the POAE, v, may be at least 0.02 or 0.05 greater than the "linear" volume fraction v', more preferably at least 0.08 or 0.1 greater, most preferably at least 0.15 or 0.2 greater than v'. In absolute terms, the actual volume fraction v is preferably 0.25 or less, more preferably 0.22 or less, yet more preferably 0.2 or 0.15 or 0.1 or 0.07 or less. It may for example be from 0.01 to 0.25, preferably from 0.05 to 0.25, more preferably from 0.05 or 0.1 to 0.2.

Thus as a result of carrying out the method of the third aspect of the invention, the concentration of the POAE in the overall fuel composition (or at least in the base fuel/POAE mixture) will preferably be as described above in accordance with the first and/or the second aspect of the invention.

According to a fourth aspect, the present invention provides a method for reducing the CFPP of a diesel fuel composition, and/or for preparing a diesel fuel composition with a CFPP at or below a desired target CFPP X, the method comprising selecting a diesel base fuel and a POAE; measuring the CFPP of mixtures of the base fuel and the POAE at 2 or more, preferably 3 or 5 or 7 or more, POAE concentrations between 0 and 100 % v/v; determining an optimal POAE concentration, or a range of optimal POAE concentrations, where the CFPP is lower than that of the base fuel alone and preferably where the CFPP reaches a minimum level; and formulating a diesel fuel composition containing the diesel base fuel and the POAE at the optimal concentration or at a concentration within the optimal range.

This method may be used in a similar fashion to that of the third aspect of the invention.

The methods of the second, third and fourth aspects of the invention may additionally or alternatively be used to adjust any property of the diesel fuel composition which is equivalent to or directly or indirectly associated with CFPP or cold flow performance generally.

A method according to the second, third or fourth aspect of the invention may form part of a process for, or be implemented using a system for, controlling the blending of a fuel composition, for example in a refinery. Such a system will typically include means for introducing a POAE and a diesel base fuel into a blending chamber, flow control means for independently controlling the volumetric flow rates of the POAE and the base fuel into the chamber, means for calculating the volume fraction of the POAE needed to achieve a desired target CFPP input by a user into the system and means for directing the result of that calculation to the flow control means which is then operable to achieve the calculated volume fraction in the product composition by altering the flow rates of its constituents into the blending chamber.

In order to calculate the required volume fraction, a process or system of this type will suitably make use of known CFPP values for the base fuel and POAE concerned, and conveniently also a model predicting the CFPP of varying concentration blends of the two according to linear blending rules. The process or system may then, according to the invention, select and produce a POAE volume fraction higher than that predicted by the linear blending model to be possible. It may use a so-called quality estimator which will provide, using a model, a real-time prediction of the CFPP of each resulting blend from available raw process measurements, such as for example the measured CFPP values and the volumetric flow rates of the constituents. More preferably such a quality estimator is calibrated on-line by making use of for example a method analogous to that described in WO-A-02/06905.

Other indicators of cold flow performance may be used instead of or in addition to CFPP values.

Methods according to the invention may thus conveniently be used to automate, at least partially, the formulation of a diesel fuel composition, preferably providing real-time control over the relative proportions of the POAE and base fuel incorporated into the composition, for instance by controlling their relative flow rates.

In accordance with the invention, use of a POAE in any of the ways described above may also embrace supplying a POAE, or a formulation containing a POAE, together with instructions for its use in a diesel fuel composition to improve or maintain the cold flow performance of the composition and/or to reduce the level of cold flow or other additives in the composition and/or to achieve a target maximum CFPP X. The POAE may be supplied as a component of a formulation suitable and/or intended for use as a fuel additive, in which case the POAE may be included in the formulation for the purpose of influencing the effects of the overall formulation on the cold flow performance of a fuel.

Other preferred features of the second, third and fourth aspects of the invention, for instance regarding the nature(s) and concentration(s) of the base fuel, the POAE and any other components of the fuel composition, may be as described above in connection with the first aspect. In particular the POAE is preferably a C₁ to C₅ alkyl ester, more preferably a methyl, ethyl or propyl (suitably iso-propyl) ester, yet more preferably a methyl or ethyl ester and most preferably the methyl ester. It is preferably used in the absence of other cold flow enhancing additives.

A fifth aspect of the invention provides a diesel fuel composition prepared, or preparable, using a method according to the second or the third aspect. This composition will suitably contain a major proportion of a diesel base fuel having an ultra low sulphur content (for example, less than 50 ppmw); and/or a CFPP (IP 309) of -6 to -10 °C.

Preferred features of the fifth aspect of the invention, for instance regarding the nature of the POAE, the diesel base fuel and any other constituents of the fuel composition, may be as described above in connection with the first aspect.

In accordance with a sixth aspect, the invention provides a method of operating a diesel engine, and/or a vehicle which is driven by a diesel engine, which method involves introducing into a combustion chamber of the engine a diesel fuel composition according to the first and/or the fifth aspect of the invention. The fuel composition may be used in this way for a purpose as referred to in connection with the second, third and/or fourth aspects of the invention, conveniently to improve the low temperature performance of the engine.

A seventh aspect of the invention provides a process for the preparation of a diesel fuel composition, such as a composition according to the first or the fifth aspect, which process involves blending a diesel base fuel with a POAE, either for the purpose of improving the cold flow performance of the composition and/or so as to achieve a POAE concentration of up to 25 % v/v, preferably more than 5 % v/v, in the overall composition.

Preferred features of the sixth and seventh aspects of the invention may be as described above in connection with the preceding aspects.

Other features of the present invention will become apparent from the following example. Generally speaking the invention extends to any novel one, or any novel combination, of the features disclosed in this specification (including the accompanying claims). Moreover unless stated otherwise, any feature disclosed herein may be replaced by an alternative feature serving the same or a similar purpose.

The example shows fuel compositions according to the present invention and illustrates the effect of a palm oil alkyl ester on the cold flow performance of a typical ultra low sulphur diesel base fuel.

### Example

The cold flow performance of various POME (palm oil methyl ester) containing diesel fuel blends according to the invention was assessed by measuring the cold filter plugging points (CFPPs) of the blends according to standard test procedure IP 309.

The base fuel used was a summer grade ultra low sulphur diesel having the properties listed in Table A. It contained no cold flow additives and no refinery additives.

**Table A**

| ***Fuel property*** | ***Test* method** | |
|---|---|---|
| Density @ 15 °C (kg/m³) | IP 365 | 827.1 |
| | | |
| Viscosity @ 40 °C | IP 71 | 2.467 |
| (centistokes) | | |
| | | |
| Distillation (°C) | IP 123 | |
| IBP | | 168 |
| 10% recovery | | 200 |
| 20% | | 214 |
| 30% | | 231 |
| 40% | | 249 |
| 50% | | 264 |
| 60% | | 279 |
| 70% | | 294 |
| 80% | | 310 |
| 90% | | 329 |
| 95% | | 345 |
| FBP | | 352 |
| | | |
| Cloud point (°C) | IP 219 | -7 |
| | | |
| Sulphur (ppmw) | ASTM D2622 | 46 |

The POME was sourced from Malaysia and had the properties listed in Table B.

**Table B**

| ***POME property*** | ***Test method*** | |
|---|---|---|
| Density @ 15 °C (kg/m³) | IP 365 | 874.2 |
| | | |
| Acid number (total) | IP 139 | 0.16 |
| (mgKOH/g) | | |
| | | |
| Iodine number | IP 84 | 52 |
| (gI₂/100g) | | |
| | | |
| Water content (ppmw) | UK 3367 | 315 |
| | | |
| Viscosity @ 40 °C | IP 71 | 4.385 |
| (centistokes) | | |
| | | |
| Distillation (°C) | IP 123 | |
| IBP | | 320.1 |
| 10% recovery | | 323.7 |
| 20% | | 324.3 |
| 30% | | 325.2 |
| 40% | | 325.4 |
| 50% | | 326.5 |
| 60% | | 327.1 |
| 70% | | 328.5 |
| 80% | | 329.7 |
| 90% | | 332.9 |
| 95% | | 336.8 |
| FBP | | 346.3 |
| | | |
| Cloud point (°C) | IP 219 | 14 |
| | | |
| Sulphur (ppmw) | ASTM D2622 | <5 |

Physical blends were prepared containing different concentrations of the POME with the base fuel. The CFPPs of these blends were then tested according to IP 309. The results are shown in Table 1 (POME concentrations are based on the volume of the overall POME/base fuel blend).

**Table 1**

| ***POME concentration (% v*/*v)*** | ***CFPP (°C)*** |
|---|---|
| 0 | -6 |
| (ie, neat base fuel) | |
| 2.5 | -7 |
| 5 | -8 |
| 7.5 | -10 |
| 10 | -10.5 |
| 12.5 | -10.5 |
| 15 | -10.5 |
| 20 | -9 |
| 30 | -4 |
| 50 | 5 |
| 100 | 13 |

These data show a marked suppression of CFPP at POME concentrations up to at least 20 % v/v. Thus the use of up to 20 % v/v POME as an additive in a diesel fuel composition can be expected to improve the cold flow performance of the composition as compared to either the base fuel or the POME alone, and the improvement is contrary to what would be expected if the cold flow performance properties of the POME and the base fuel were purely additive.

By way of comparison, it has been found that blends containing rapeseed methyl ester, another fatty acid methyl ester (FAME) which is in some ways analogous to POME, show a linear increase in CFPP with increasing FAME concentration. Other fatty acid alkyl esters have demonstrated similar trends in a range of diesel base fuels, acting to increase the CFPP (and hence worsen cold flow performance) at any concentration. This makes the effect observed with palm oil alkyl esters even more surprising.

## Claims

1. A diesel fuel composition containing a diesel base fuel and a palm oil alkyl ester (POAE), wherein the POAE concentration is up to 25 % v/v based on the overall composition.

2. A diesel fuel composition according to claim 1, wherein the POAE concentration is greater than 5 % v/v based on the overall composition.

3. A diesel fuel composition according to claim 1 or claim 2, wherein the POAE is a palm oil methyl, ethyl or iso-propyl ester.

4. Use of a POAE in a diesel fuel composition, for the purpose of improving the cold flow performance of the composition.

5. Use according to claim 4, wherein the POAE is.used in an amount sufficient to reduce the cold filter plugging point (CFPP) of the composition by at least 3 °C compared to its value prior to addition of the POAE.

6. Use according to claim 4 or claim 5, wherein the POAE is used at a concentration of from 5 to 20 % v/v based on the overall fuel composition.

7. Use according to any one of claims 4 to 6, wherein the fuel composition contains less than 50 ppmw of additional cold flow additives.

8. Use of a POAE in a diesel fuel composition, for the purpose of reducing the level of cold flow additives in the composition.

9. Use according to any one of claims 4 to 8, wherein the POAE is a palm oil methyl, ethyl or iso-propyl ester.

10. A method for preparing a diesel fuel composition with a CFPP at or below a desired target X, the method comprising selecting a diesel base fuel and a POAE; measuring the CFPP of mixtures of the base fuel and the POAE at two or more POAE concentrations between 0 and 100 % v/v; determining an optimal POAE concentration, or a range of optimal POAE concentrations, where the CFPP is lower than that of the base fuel alone and preferably where the CFPP reaches a minimum level; and formulating a diesel fuel composition containing the diesel base fuel and the POAE at the optimal concentration or at a concentration within the optimal range.
